

Sept. 6, 1932.

E. PLAYER

1,876,073

PROCESS OF CASTING LIGHT METALS IN SAND MOLDS

Filed Sept. 19, 1929



*Edward Player*  
INVENTOR.

BY  
*Hough & Ward*  
ATTORNEYS.

## UNITED STATES PATENT OFFICE

EDWARD PLAYER, OF ASTLEY, ENGLAND, ASSIGNOR, BY MESNE ASSIGNMENTS, TO  
MAGNESIUM DEVELOPMENT CORPORATION, A CORPORATION OF DELAWARE

## PROCESS OF CASTING LIGHT METALS IN SAND MOLDS

Application filed September 19, 1929, Serial No. 393,844, and in Germany September 19, 1928.

This invention relates to the casting of metals in sand molds.

When casting metals into sand molds it is generally considered necessary, especially in the case of complicated castings, to employ so called "chills" in various sections of the mold, i. e. to insert metal plates in the inner surface of the mold which on contacting with the molten metal cause a more rapid cooling of the casting in that particular section, thus preventing the setting up of internal stresses and the formation of cracks and similar defects in the casting on further cooling. The necessity for employing chills in sand molds is particularly pronounced in the casting of light metals such as aluminum and magnesium, these metals having a stronger tendency to warp and to crack owing to their comparatively high shrinkage. As the molten metal does not easily rest on the chills when the latter are cold it is further necessary to heat the chills before filling the mold with metal so as to ensure a flawless surface of the castings in these places. This heating is generally effected by means of a suitable burner or blow-pipe, the jet being directed successively on the different chills.

While this method, although apparently primitive, yields very good results in the case of smaller castings, it has proved far from reliable when larger castings provided, sometimes, with from fifty to several hundred chills, are concerned. In such cases, the surface of the casting frequently displays blow-holes and similar defects in the place of the chills. Attempts to remove these deficiencies of the method by a more intense heating of the chills and by the application of various blackwashes were of small avail and did not result in rendering the production of perfect castings reliable on a commercial scale.

These difficulties, while existing also to some extent when casting aluminum, appear seriously enhanced in the case of magnesium and its alloys, which are usually cast into green sand molds impregnated with volatilizable protective substances, as a more intense heating of the chills causes these substances to evaporate in the sections of the sand sur-

rounding the chills and this frequently gives occasion to a detrimental reaction between the sand of the mold and the molten metal. Moreover, magnesium and its high percentage alloys are liable to react chemically with any sensible moisture condensed on the surface of chills. 55

A closer investigation of the causes of these difficulties by applicants has now revealed that they must be attributed to differences in the temperature of the various chills. These differences arise from the successive heating of the individual chills by means of burners or the like, which procedure allows the chills first heated to cool down to lower temperatures, mostly by radiation, while other chills are still being heated. On closing the mold the moisture contained in the sand surrounding the hottest chills evaporates and pervading the interior of the mold, is condensed on such chills as, although still warm, have cooled down in the meantime. On contact with the molten metal, these condensations of moisture give rise to blow-holes or similar defects in the surface of the casting. 75

It follows from the result of these investigations that the heating of the chills should be carried out in such a manner that all the chills in the mold are simultaneously and uniformly heated. 80

Experiments along these lines have resulted in the production of perfect light metal castings, even when very large and provided with a great number of chills. They have further elicited the fact that the temperature range within which the chills must be heated so as to ensure perfect castings, is much wider than was hitherto anticipated, as long as the differences in temperature of the individual chills are kept within narrow limits. 85 90

A suitable way of carrying the present invention into practice consists in passing a current of sufficiently heated air through the closed mold for some time before casting until the chills have uniformly assumed the desired temperature which is preferably between about 50 and 100° C. The heated air is preferably introduced into the mold by means of a pipe whose nozzle is inserted into 100

one of the apertures of the mold (such as risers or runner bushes).

In the accompanying drawing a vertical section of a suitable apparatus for carrying out the present invention is represented in a diagrammatic manner. *a* designates the sand mold, whereas *b* represents the free space corresponding to the outlines of the finished casting. *c* are chill plates inserted at two points of the mold where the nature of the casting requires enhanced cooling. One end of a suitable mouth-piece *e* is detachably fitted to one of the gates *d* of the mold, whereas its other end is connected with the tap *g* of a suitable air heating device (not shown) by means of a flexible tube *f*. The heated air is supplied to the mold by means of the mouth piece *e* and, after circulating in the hollow space *b*, issues from the mold partly by the free gate *d*, partly by the crevices in the sand of the mold. When the chill plates *c* have uniformly attained the desired temperatures, the mouth piece *e* is removed from the mold which is thereupon immediately filled with the molten metal in the usual manner.

I claim:

In a process of casting light metals in green sand molds provided with a plurality of local chill plates the preliminary step of simultaneously and uniformly heating said chill plates to a temperature within the range between about 50 and 100° C., by passing a current of heated air through the mold for some time prior to casting.

In testimony whereof I have hereunto set my hand.

EDWARD PLAYER.

40

45

50

55

60